

# United States Patent [19]

Binnersley et al.

[11] Patent Number: 4,947,897

[45] Date of Patent: Aug. 14, 1990

[54] **METHOD FOR PRODUCING A FABRIC MADE FROM THERMOPLASTIC MELT IMPREGNATED TOW**

[75] Inventors: **Edwin K. Binnersley, Wilmington, Del.; James M. Batman, Coopersburg, Pa.**

[73] Assignee: **E. I. du Pont de Nemours and Company, Wilmington, Del.**

[21] Appl. No.: 301,399

[22] Filed: Jan. 24, 1989

## Related U.S. Application Data

[62] Division of Ser. No. 848,866, Apr. 7, 1986, Pat. No. 4,816,327.

[51] Int. Cl. 5 ..... D03D 47/34; D03D 47/14

[52] U.S. Cl. ..... 139/445; 139/452

[58] Field of Search ..... 139/11, 35, 97, 98, 139/100, 443, 445, 452, 420 R; 428/225

## References Cited

### U.S. PATENT DOCUMENTS

3,503,106 3/1970 Port et al. ..... 139/11  
3,575,217 4/1971 Pfarrwalter ..... 139/452

|           |         |                         |             |
|-----------|---------|-------------------------|-------------|
| 3,587,661 | 6/1971  | Golobart .....          | 139/445     |
| 3,626,989 | 12/1971 | Held .....              | 139/97      |
| 3,930,091 | 12/1975 | Lewis et al. .....      | 428/198     |
| 3,993,726 | 11/1976 | Moyer .....             | 264/174     |
| 4,160,057 | 7/1979  | Kogan et al. .....      | 139/420 R X |
| 4,235,262 | 11/1980 | Ushiro .....            | 139/452     |
| 4,640,861 | 2/1987  | Binnersley et al. ..... | 428/294     |
| 4,816,327 | 3/1989  | Binnersley et al. ..... | 428/225     |

Primary Examiner—Andrew M. Falik

## [57] ABSTRACT

Formable twistless woven precursor fabrics, especially in satin or basket weave, made from warp and weft flat tape of fiber reinforced thermoplastics on a power driven loom. The weft tape is supplied in a twistless manner from a rotatable package that is driven in synchronism with the feeding mechanism and a finite tension on the tape is maintained so that a line drawn parallel to the surface of and perpendicular to the longitudinal axis of each of the warp and weft tapes is in the plane of the fabric throughout the fabric. The warp and weft tapes have edges that abut substantially throughout the fabric.

1 Claim, 2 Drawing Sheets







**METHOD FOR PRODUCING A FABRIC MADE  
FROM THERMOPLASTIC MELT IMPREGNATED  
TOW**

This is a division of application Ser. No. 848,866, filed 4/7/86 U.S. Pat. No. 4,816,327.

**BACKGROUND OF THE INVENTION**

This invention relates to woven fabrics, and more particularly, it relates to fabrics woven from flat tape or tow of fiber reinforced plastic material.

Fiber-reinforced plastic structures have been used for many years with increasing success because of their high strength, light weight and ease of fabrication compared to the wood or metal structures which they replace. Fibers such as glass, carbon and aramid are popular as reinforcement, and thermosetting resins such as polyester, phenolic and epoxy are common polymeric matrices.

Polymeric materials reinforced with continuous filaments are used as precursors for highly-stressed parts such as aerospace components requiring the highest possible strength with the lowest possible weight. Non-uniformity of the materials comprising such parts requires that the parts be over-constructed so that the weakest will surpass the service requirements. More uniform precursor materials would yield parts having less variation in properties and would permit constructing such parts more efficiently to design criteria.

Weaving, to which this invention applies, comprises forming a fabric on a loom by interlacing warp and weft threads. The prior art includes many techniques for feeding the weft threads through the warp. Conventionally the weft is taken from a stationary package with an "over the end of the package takeoff" which results in twist being formed in the weft.

When weaving such reinforced tape in satin weave and basket weave fabric constructions under such weaving conditions the weft tape will likely have twist formed during the weaving operation. Such twist would represent an undesirable nonuniformity in the fabric. Therefore, the production of woven fabrics from tape of fiber reinforced plastic without such twisting would be highly desirable.

**SUMMARY OF THE INVENTION**

This invention provides a method for producing woven fabrics from flat tape of fiber reinforced plastic on a power driven loom having warp and weft directions. The weft tape is supplied from a rotatable package and is fed in synchronism with the device that feeds the tape through the weft and is tensioned and guided to maintain the tape in the plane of the fabric throughout the fabric without twist. The warp and weft tapes are arranged so that a line parallel to the surface of each of the tapes and perpendicular to its longitudinal axis is in the plane of the fabric in the warp and weft directions throughout the fabric.

**BRIEF DESCRIPTION OF THE DRAWING**

FIG. 1 is a schematic elevation of the weft feeder mechanism used in conjunction with a loom to perform the method of this invention.

FIG. 2 is an enlargement of a tensioner of FIG. 1.

FIG. 3 is a schematic representation of an 8-harness satin fabric made using the method of this invention.

**DETAILED DESCRIPTION OF THE  
ILLUSTRATED EMBODIMENT**

Referring to FIG. 1, a loom generally designated as 5 10 is fed from a warp set of fiber reinforced plastic tapes 14 wound without twist on rotatably driven beam 12. The tapes 14 pass in the usual well known manner toward a rotatably driven fabric takeup beam 30 which winds the woven fabric 32 thereon. A flat fiber reinforced plastic tape 18 used for the weft direction of the fabric is withdrawn from a rotatable supply package 19 by a pair of nip rolls 20,21 into an accumulation loop and from the loop fed to the rapier 28 of the loom through guides 15,17 tensioners 22,23, and feeder guide 15 positioner 24. The weft tape 18 is then interlaced through the warp tapes 14 in the usual manner to form the fabric 32. Feed apparatus 19, 20, 21 is mounted to a frame (not shown).

The nip roll 20 is driven by variable speed motor 20 (Zero Max-model M-2) 25 via belt 27. The motor speed is adjusted to synchronize the feeding means (nip rolls 20,21) with the movement of rapier 28, i.e., the motor speed is set according to rapier movement so that a loop is provided between guide 15 and feed rolls 20, 21.

The tensioners 22,23 are comprised of a center post 50, attached to the lay of the loom 10a. The center post has a slot 51 through which tape 18 passes. Two tension discs 52,53 are positioned by post 50 and disc 52 is biased toward disc 53 by spring 55 located between disc 52 and stop nut 50a on post 50.

Referring now to FIG. 3, a small portion of the fabric 30 of this invention is shown schematically in perspective to illustrate what is meant by twistless warp or weft tape. More particularly, as illustrated, a line 40a is drawn parallel to the surface 41 of weft tape 18 and perpendicular to the longitudinal axis 42 of the tape. If the weft tape is flat throughout the fabric and without twist, then line 40a drawn at any point along the weft will be in the plane of the fabric. The same applies to the warp tapes 14 using a line 40 perpendicular to longitudinal axis 42a.

**EXAMPLE**

Eight woven fabrics are prepared using an IWER Series 1500 Rapier Loom. Each fabric is woven from warp and weft tapes and is of woven constructions as detailed in Table I. The tapes have nominal thickness of 5 to 12 mils and a width of about 3/16" and comprise 50 reinforcing fibers such as carbon, Kevlar and glass impregnated with a thermoplastic resin. The particular resin used was a copolyamide from hexamethylene diamine, bis(para-aminocyclohexyl)methane, isophthalic acid and terephthalic acid disclosed by Chang in U.S. patent application Ser. No. 819,562 filed Jan. 17, 1986.

**TABLE I**

| Sample<br>No. | Weave<br>Type   | Fiber<br>Reinforc. | Picks/in |      | Weight<br>Oz/yd <sup>2</sup> |
|---------------|-----------------|--------------------|----------|------|------------------------------|
|               |                 |                    | Warp     | Weft |                              |
| A             | 4 x 4 basket    | graphite           | 5.9      | 11.4 | 6.5                          |
| B             | 4 Harness satin | graphite           | 5.8      | 11.5 | 6.3                          |
| C             | 4 x 4 basket    | Kevlar             | 6.1      | 7.2  | 6.2                          |
| D             | 4 Harness satin | Kevlar             | 6.0      | 7.1  | 6.2                          |
| E             | 4 x 3 basket    | Glass              | 3.6      | 4.8  | 10.0                         |
| F             | 4 Harness satin | Glass              | 4.0      | 4.8  | 10.0                         |
| G             | 8 Harness satin | Kevlar             | 8.0      | 7.8  | 7.7                          |
| H             | 8 Harness satin | Glass              | 6.0      | 5.8  | 13.6                         |

In Samples G and H the edges of the tapes in the warp and weft directions were abutting and exhibited no twist.

An 8-harness satin fabric, made of Sample G above, was formed into a composite by heating 8 layers of the fabric in an infra-red oven between two glass layers precoated with Fre kate 33 to a temperature of 370° C. The layers were then placed on top of a 6-inch hemispherical mold and the perimeter of the layers was securely clamped. The molding conditions were 150° C. at a pressure of 30 tons. The mold was then cooled to 110° C. under pressure and opened. The period for molding and cooling was about 20 minutes.

A series of plaques formed of plies of 8-harness satin woven fabric of sample G were made as detailed in Table II.

TABLE II

| No. Plies                    | 6                 | 16          | 6           |
|------------------------------|-------------------|-------------|-------------|
| Size of Ply                  | 6" × 6"           | 6" × 6"     | 6" × 6"     |
| Orientation                  | 0/90              | [90/0]4S    | 0/90        |
| Laminate Thickness           | 43 mils<br>(.043) | 114 mils    | 42 mils     |
| Consolidation<br>Conditions* |                   |             |             |
| TEMP.                        | 295-305° C.       | 295-305° C. | 295-305° C. |
| PRESSURE                     | 305 psi           | 305 psi     | 305 psi     |

30

TABLE II-continued

| TIME | 30 min. | 30 min. | 30 min. |
|------|---------|---------|---------|
|------|---------|---------|---------|

\*Cooled under pressure

The fabric, which consists of tape the surfaces of which remain parallel to the plane of the fabric throughout the fabric without twist, when formed into composites such as laminates or molded parts by thermoforming processes demonstrated conformability and uniformity.

We claim:

1. A method for producing woven fabrics from flat warp and weft tapes of continuous filaments impregnated with polymer on a power driven loom having warp and weft directions comprising: feeding weft tapes in a twistless manner from a rotatable supply package to said loom with variable speed feeding means; inserting said weft tapes in the weft direction through a warp shed of said warp tapes with a driven movable rapier, said variable speed feeding means being synchronized with the movement of said rapier; and tensioning and guiding said warp and weft tapes to maintain each of said warp and weft tapes in such a manner that a line parallel to the surface of and perpendicular to the longitudinal axis of each of the tapes is in the plane of the fabric throughout the fabric, said warp and weft tapes having edges that are abutting substantially throughout the fabric.

\* \* \* \* \*

30

35

40

45

50

55

60

65